

## UNITED STATES PATENT OFFICE

1,967,569

## PRINTING

John Elton Cole, Wilmington, Del., assignor to  
E. I. du Pont de Nemours & Company, Wilming-  
ton, Del., a corporation of Delaware

No Drawing. Application January 25, 1933,  
Serial No. 653,548

## 19 Claims. (Cl. 8—6)

This invention relates to the art of textile printing, and more particularly to the preparation of improved printing pastes and vat dye pastes. Specifically, it contemplates a novel type of printing assistant for use in pastes containing indigoid, and especially thioindigoid dyes.

Textile printing differs from dyeing in that the color or colors applied are confined to certain parts of the material, thus producing different designs or patterns. At the present time, the most extensive textile printing is done with cylinders or roll printing machines. The fundamental principles in this art are simple and comprise passing the cloth to be printed under some tension and pressure over an intaglio metal roll, the engraving of which is filled with a printing paste. After leaving the printing machine, the printed cloth is passed into a drier. This dries the printing paste on the cloth in its proper place and prevents the dye from spreading to other portions of the fabric. In order to complete the printing, the cloth, after leaving the drier, is passed into a steam ager for a period of a few minutes, during which time the vat color undergoes reduction and passes to the fiber. The fabric is then subjected to oxidizing conditions which may include passing it into a steeping bath, usually of water or water containing an oxidizing agent. Any excess color is washed off in a soap solution with which the textile material is treated following the steeping.

The composition of vat dye printing pastes may vary widely with different dyes and manufacturers, but usually consists of a mixture of an unreduced vat dye, a strong reducing agent such as, for example, sodium hydrosulfite or sodium formaldehyde sulfoxylate, an alkali and a thickening agent. The thickening agent is usually a gum (for instance, British gum), starch, or both. The printing paste is usually prepared by mixing a dye paste or pastes with the other ingredients, said other ingredients being in the form of a gummy mixture generally called a printing gum. The dye pastes are essentially finely divided suspensions of the dye, with or without a dispersing agent. In general, any substance which is responsible for results in textile printing which show an improvement over a water suspension dye paste may be called a printing assistant. Printing assistants may be added to the dye paste or to the printing gum or to the printing paste, as desired.

It is an object of the present invention to produce improved results in textile printing. Other objects are to produce improved printing pastes, improved printing gums, improved dye pastes

and improved printing assistants and, in general, to improve the art of textile printing. A further and more specific object is to produce improved results in printing indigoid dyes, and especially thioindigoid dyes. Other objects will appear 60 hereinafter.

These objects are accomplished according to the present invention whereby formates or compounds capable of yielding formates under the conditions of printing are used as printing assistants. These compounds may be used alone or in conjunction with other printing assistants.

While the invention is susceptible to considerable variation and modification in the manner of its practical application, particularly as regards 70 the nature and proportions of materials used, and the exact method of procedure, the following examples, in which the parts are by weight, will illustrate the practice of the invention.

## Example I

75

Twenty parts of a dye paste containing 10% formamide and 10% 6:6'-diethoxy thioindigo were mixed with 80 parts of a printing gum containing:

80

|                                 | Parts   |
|---------------------------------|---------|
| Potash                          | 9.1     |
| Sodium formaldehyde sulfoxylate | 6.6     |
| Glycerine                       | 10.0    |
| Thickener                       | 54.3 85 |

The thickener employed was prepared by mixing:

Parts

|                              |     |    |
|------------------------------|-----|----|
| Wheat starch                 | 1.0 | 90 |
| British gum                  | 3.0 |    |
| Water                        | 4.0 |    |
| Gum tragacanth (6% solution) | 1.0 |    |

The resulting printing paste was printed on a textile material and developed in the usual manner. The prints were noticeably stronger and brighter than those obtained from an exactly similar mixture without the addition of the formamide.

## Example II

100

Twenty parts of a dye paste containing 10% 6:6'-diethoxy thioindigo and 10% sodium formate were mixed with 80 parts of a printing gum similar to the one mentioned in Example I, and this mixture was printed on a textile material in the usual manner. The printing obtained was stronger and brighter than the one obtained from an exactly similar mixture in the absence of sodium formate.

105

110

*Example III.*

Twenty parts of a dye paste containing about 12.5% of 4:4'-dimethyl-6:6'-dichlor thioindigo and 10% of formamide were mixed with 80 parts of a printing gum and printed on a textile material in the usual manner. The resulting prints were about 10% stronger than those obtained from a similar mixture in the absence of the formamide.

*Example IV*

Twenty parts of a dye paste containing 20% of 5:5'-dichlor-7:7'-dimethyl thioindigo and 10% formamide were mixed with 80 parts of printing gum and printed on a textile material. The prints obtained were about 10% to 15% stronger than those obtained from a similar mixture in the absence of the formamide.

*Example V*

Twenty parts of a dye paste containing 20% of bis-beta-naphthionaphthene indigo and 10% of formamide were mixed with a printing gum containing potash, sodium formaldehyde sulfoxylate and glycerine. The resultant mixture was printed on a textile material and developed in the usual manner. The prints obtained were stronger than those obtained from a similar mixture without the addition of the formamide.

*Example VI*

Twenty parts of a dye paste containing 10% of tetra-bromo-indigo and 10% of formamide were mixed with 80 parts of a printing gum, printed and developed in the usual way. The resultant prints were noticeably stronger and brighter than those obtained from a similar mixture in the absence of the formamide.

Instead of tetra-bromo-indigo, a dye paste containing corresponding proportions of 4:4'-dichloro-5:5'-dibromo-indigo may be used with improved results.

*Example VII*

A printing gum was prepared by mixing together:

|                                                                               | Parts |
|-------------------------------------------------------------------------------|-------|
| Formamide                                                                     | 4.0   |
| Potash                                                                        | 9.1   |
| Sodium formaldehyde sulfoxylate                                               | 6.6   |
| Glycerine                                                                     | 10.0  |
| Thickener (having the approximate composition of that described in Example I) | 50.3  |

The resultant product was incorporated with 20 parts of a 10% commercial paste of 6:6'-diethoxy thioindigo, and the printing paste thus obtained was printed on a textile material in the usual manner. The prints obtained were stronger and brighter than those obtained from an exactly similar mixture in the absence of formamide.

According to procedures similar to those described in the examples, other dye pastes, printing pastes and printing gums, giving improved results in printing, may be obtained. Insofar as is known, the application of the invention gives improved results in printing any indigoid dyes. Especially desirable results have been obtained in printing the thioindigo dyes, such as those described in the examples, and mixtures thereof.

The printing assistant preferably used in accordance with the invention is formamide. It will be recognized, when vat dye pastes containing formamide are added to a strongly alkaline medium like the printing gums used in the art, that alkali formates and ammonia will most prob-

ably be formed. As a general rule, the salts of formic acid added to the printing mixtures are as efficient printing assistants as formamide on an equal molal basis. Where a formate is used as such, it is preferable to use the soluble salts of formic acid, particularly the alkali metal formates.

As already indicated, the assistants may be added advantageously to the color paste, or they may be mixed with the printing gum before or after the addition of the color. It is possible to add up to about 10% of sodium formate, for instance, to a dye paste. Such a procedure is not very practical, however, in most cases, due to the tendency of such semi-colloidal suspensions to jell upon the addition of salts. Therefore, when it is desired to add the assistant to the dye paste, it is usually found to be more convenient to add the formamide since it has little effect on the physical nature of the paste. In case it is desired to add the assistant to the printing gum, it is generally more convenient to use the salts themselves. If sufficient alkali is present, formic acid could equally well be used in the printing gum.

The amount of printing assistant may vary within relatively wide limits but may ordinarily be varied directly with the amount of dye. Empirical tests can usually be made to determine the optimum amount of printing assistant for any given dye. Very satisfactory results are obtained with the proportions of printing assistant described in the examples, but greater or less amounts may be employed, if desired. If salts of formic acid are used directly in the printing gum, there is practically no limit to the amount which can be used without deleterious effect. If formic acid or formamide is used, however, care must be taken that there is sufficient alkali present to neutralize the assistant and still be alkaline enough to print well. If formamide is used, too large an excess is undesirable due to the large amount of ammonia evolved. The amounts of the various assistants used in the examples give good results without requiring adjustment of the alkali content of the printing gum. Less than the designated amounts could be used to advantage but the improvement is not so marked. In general, the amount of assistant should preferably be within the range of about 1.0% to about 20.0%, on the basis of the weight of the dye paste. Especially desirable results have been obtained in the use of about 10% of assistant, based on the weight of the dye paste.

The process of the invention gives particularly valuable results with regard to the fullness and brightness of shade when the substratum upon which the color is printed is mercerized cotton. Good results may also be obtained in printing other cotton materials and, in general, materials which may be printed with vat colors, including viscose rayon and other fibers, fabrics and yarns.

As previously indicated, the invention is particularly advantageous in that the presence of assistants of the character described in the printing paste makes possible the production of prints of superior strength and brightness to those obtained from a similar printing paste from which the assistant has been omitted. The use of formamide is of special advantage in that it may be incorporated directly with the dye paste and has no harmful effect thereon, so that the resultant paste may be marketed as such and re-

- quires only mixing with the printing gum for use in printing.
- Throughout the specification and claims it will be understood that the term "indigoid" is intended to include not only indigo and dyes of the indigo series, but also thioindigo and other dyes of this type, as, for example, dyes falling within the general formula and classification given by G. von Georgievics and E. Grandmougin in "A Textbook of Dye Chemistry", 428, 1920.
- As many apparently widely different embodiments of this invention may be made without departing from the spirit and scope thereof, it is to be understood that I do not limit myself to the specific embodiments thereof except as defined in the following claims.
- I claim:
1. A dye paste comprising a water insoluble vat dye and a compound selected from the group consisting of formates and substances capable of yielding formates under the conditions of printing.
  2. A printing paste comprising an unreduced vat dye and having an addition thereto of a compound selected from the group consisting of formates and substances capable of yielding formates under the conditions of printing.
  3. A dye paste comprising a water-insoluble indigoid dye and a compound selected from the group consisting of formates and substances capable of yielding formates under the conditions of printing.
  4. An indigoid printing paste comprising an unreduced indigoid dye having an addition thereto of a compound selected from the group consisting of formates and substances capable of yielding formates under the conditions of printing.
  5. An indigoid printing gum for use in printing unreduced indigoid dyes, said printing gum including a compound selected from the group consisting of formates and substances capable of yielding formates by reaction with an alkali.
  6. A water-insoluble indigoid dye printing paste containing an alkali metal formate.
  7. A dye paste comprising a water-insoluble indigoid dye and formamide.
  8. A dye paste comprising a water-insoluble thioindigoid dye and a compound selected from the group consisting of formates and substances capable of yielding formates under the conditions of printing.
  9. A thioindigoid printing paste comprising an unreduced thioindigoid dye and having an addition thereto of a compound selected from the group consisting of formates and substances capable of yielding formates under the conditions of printing.
  10. A thioindigoid printing gum for use in printing an unreduced thioindigoid dye, said printing gum including a compound selected from the group consisting of formates and substances capable of yielding formates by reaction with an alkali.
  11. An unreduced thioindigoid dye printing paste containing an alkali metal formate.
  12. A dye paste comprising an unreduced thioindigoid dye and formamide.
  13. A dye paste comprising an unreduced thioindigoid dye and about 10% by weight of formamide.
  14. A printing paste containing 6:6'-diethoxy thioindigo and an alkali metal formate.
  15. A process which comprises printing textiles with a vat dye printing paste of the type in which the dye is originally water-insoluble, in the presence of a formate.
  16. A process of printing textiles which comprises adding to a paste containing a water-insoluble indigoid dye and other customary ingredients a compound selected from the group consisting of formates and substances capable of yielding formates under the conditions of printing, and thereafter using the compounded paste in printing.
  17. A process of printing textiles which comprises adding to a paste containing an unreduced thioindigoid dye and other customary ingredients a compound selected from the group consisting of formates and substances capable of yielding formates under the conditions of printing, and thereafter using the compounded paste in printing.
  18. A process which comprises printing textiles with a printing paste containing an unreduced indigoid dye and an alkali metal formate.
  19. A process which comprises printing textiles with a printing paste containing an unreduced thioindigoid dye and an alkali metal formate.
- JOHN ELTON COLE. 125
- 55 130
- 60 135
- 65 140
- 70 145